

Patented Jan. 8, 1929.

1,698,098

# UNITED STATES PATENT OFFICE.

NOAK VICTOR HYBINETTE, OF WILMINGTON, DELAWARE.

## HEAT-ENDURING METAL.

No Drawing.

Application filed July 12, 1924. Serial No. 725,692.

This invention relates to heat-enduring metals, and particularly to alloys which resist to a material extent the effect of oxygen and other deteriorating influences under high 5 temperatures, particularly the influence of alkali. Such alloys have numerous uses in the arts and are desirable especially where conditions exist which tend to cause the rapid destruction of metals heretofore available for such purposes.

The basis of the invention is an alloy of iron, nickel and chromium. Alloys of these elements have been known heretofore and are used for various purposes. So far as 15 they meet the conditions under which they are used the alloys are satisfactory but they are useless in many cases because their endurance to oxidation, and particularly to the influence of alkalies, is relatively limited.

20 I have discovered that alloys containing these elements in certain limited proportions are much more resistant to deterioration at high temperatures than alloys heretofore known, particularly deterioration by alkali

25 at high temperatures, and that an alloy containing these elements in proportions corresponding to the atomic weights of the elements has the highest degree of endurance under adverse conditions. Such an alloy

30 which I have found valuable consists of 33 per cent iron, 36 per cent nickel, and 31 per cent chromium, approximately, and is unaffected to any material extent by exposure to air or furnace gases and alkali salts at

35 temperatures as high as 2100° F. Any oxidation resulting from such exposure involves the formation merely of a skin coating of oxide which is tough and adherent and protects the underlying metal from fur-

40 ther oxidation. This resistivity to alkali becomes noticeable with 18% nickel and 28% chromium and the remainder mainly iron, and shows a pronounced diminution with over 40% nickel, over 40% chromium and 45 less than 20% iron.

I have studied particularly the effect of alkalis upon such alloys as well as upon alloys of iron, nickel and chromium, such as have been known heretofore. The deterioration of the heretofore known alloys in the presence of alkalis has been observed and ascribed generally to causes other than the presence of alkali. I find, however, that the alkali is almost always present in sufficient 50 quantity to be of considerable importance and attacks the metal, combines therewith

and acts apparently as a catalyst so that oxidation is rapid and destruction of the metal follows quickly. The effect of the alkali does not depend upon direct contact 60 thereof with the metal although deterioration is more rapid where the alkali is applied to the metal. In a furnace in which alkali is present as vapors it causes rapid oxidation of the alloy. 65

The compositions of heat resisting alloys heretofore generally used, for instance, an alloy containing 80 per cent of nickel and 20 per cent of chromium, or one containing 50 per cent of nickel, 18 per cent of chromium 70 and 20 per cent of iron, or an alloy containing 35 per cent of nickel, 20 per cent of chromium, and 45 per cent of iron, or an alloy containing 30% chromium with little or no nickel and the rest iron, will, when heated 75 electrically to about 2000° F. in the presence of air, lose approximately one milligram of metal per square centimeter in twenty-four hours. If a small quantity of soda ash is applied to the surface of these metals in the proportion of five tenths of a milligram per 80 square centimeter, the oxidation is increased to from 10 to 100 milligrams per square centimeter. The mere introduction of a similar amount of soda ash in the furnace but not in contact with the metal results in approximately the same rate of acceleration of the oxidation by the vapors acting on the alloy. 85

On the other hand, the new alloy which I have herein described can be heated almost indefinitely to the temperature and under the conditions mentioned without material loss by oxidation. Even in the presence of sodium or other alkalies there is no material amount of oxidation or other destruction of 90 the metal. The alloy is, therefore, particularly useful in connection with operations requiring prolonged heating in the presence of oxidizing or furnace gases, and especially where alkalies contact with the metal or are present in the atmosphere to which it is subjected. 95

The atomic proportions mentioned are not absolutely essential to the accomplishment of the purpose of the invention and can be varied to a limited extent depending upon the particular use for which the alloy is intended. The physical characteristics of the metal will vary greatly with the nickel content but its endurance of the deteriorating influences of alkali salts does not materially change if the proportions of the elements are main- 100

tained within the limits hereinafter mentioned. The nickel content of the alloy can be reduced to approximately 20 per cent without impairing its endurance to any extensive degree, and I have found that an alloy containing 50 per cent of iron, 20 per cent of nickel and 30 per cent of chromium has marked endurance in the presence of alkalis and also the highest physical strength at 10 high temperatures. It will withstand the effect of an oxidizing atmosphere at a temperature of about 2100° F. for an almost indefinite time.

The alloy with about 35% nickel has practically the highest resistivity to alkali but is not so strong. The chromium content can be varied from about 28 to 40%, but in general there is little gained by using more than about 30 to 32 per cent.

20 My invention primarily consists, therefore, in an alloy of iron, nickel and chromium, in which the chromium content is always approximately 30 per cent and in which the nickel varies from 18 to 40 per cent with corresponding proportions of iron. Such an alloy meets all of the requirements for many uses in which the alloy is subjected to oxidation and other deteriorating influences. Its characteristics can be modified, however, 25 without destroying the properties mentioned to make it suitable for other purposes.

The alloys described are somewhat hard and brittle and cannot be rolled and drawn satisfactorily. It is possible, however, to 30 modify the hardness of the metal by additions of cobalt or copper. Cobalt is generally assumed to impart to such alloys the same properties as nickel does, but this is not true in the present case. For example, the addition of 35 from one to 10 per cent of cobalt softens the alloy appreciably and imparts a finely grained structure. Copper is usually considered to be detrimental to alloys containing chromium and nickel, but the alloys described can be 40 modified by additions of from five tenths to five per cent of copper without reducing the enduring properties. The copper serves the same purpose as cobalt in softening the metal and is a cheaper agent for that purpose.

50 Where great mechanical strength is requisite the addition of copper and cobalt is to be avoided as an amount in excess of one tenth of one per cent of copper reduces the strength materially. As much as 3 per cent of cobalt can be used, without reducing the strength materially.

The alloys, either with or without copper or cobalt, can be modified by the presence of varying proportions of carbon and silicon.

55 The presence of the usual amounts of these elements in the alloys does not affect their properties materially for certain purposes. For rolling and drawing, however, silicon and carbon are undesirable and should be reduced 60 to the lowest practicable proportions. Both

of these elements tend to make the metal hard and brittle.

As specific examples of the preferred compositions an alloy for castings having the highest possible endurance to the effect of 70 oxygen and alkali should contain, in addition to iron, the following elements in approximately the proportions mentioned:

|           | Per cent. |
|-----------|-----------|
| Chromium  | 30        |
| Nickel    | 35        |
| Carbon    | 1.5       |
| Silicon   | 1         |
| Manganese | .5        |
| Aluminum  | .5        |

In addition the metal may contain copper 85 1% or cobalt 1 to 10%. The addition of the latter elements is optional because these elements do not influence the endurance of the metal and they are added only to ensure 90 against brittleness. A reduction in the amount of carbon, silicon and aluminum will also soften the metal. The chromium and nickel content can be increased to approximately 40 per cent of each before a very decided decrease in the resistivity of the metal to corrosion is noticeable. However, such increase is not desirable as it increases the cost 95 of the alloy without corresponding advantages.

This alloy has the peculiar property of forming under oxidizing conditions in the presence of alkali a tough adherent surface of oxide having the consistency of graphite. 100 The oxide coating adheres to the metal in spite of repeated heating and consequently protects the surface of the metal from the further action of oxygen or other deteriorating elements. Receptacles made of this alloy and provided with such a surface coating are useful 105 for many chemical purposes in addition to handling of alkali compounds, such, for example, as the melting of aluminum. In the latter use care should be taken that the temperature does not rise above the point where the aluminum reduces the oxide. For lead baths and many other purposes it is superior to other alloys, even though its peculiar resistivity to alkali is not taken advantage of. 110

115 For mechanical structures requiring great strength but not so great resistivity to alkali I prefer an alloy containing, in addition to iron, the following elements in the proportions mentioned:

|           |            |          |                 |
|-----------|------------|----------|-----------------|
| Chromium  | between 28 | and 32%, | preferably 30%  |
| Nickel    | between 18 | and 22%, | preferably 20%  |
| Carbon    | between 1  | and 2%,  | preferably 1.5% |
| Silicon   | .5 to      | 2%,      | preferably 1%   |
| Aluminum  | .1 to      | 2%,      | preferably .5%  |
| Manganese | 0 to       | 5%,      | preferably .5%  |

120 It is understood that in this and the composition previously described the amount of iron is proportionate to complete the composition.

125 For heat-treatment containers the composition last described may be used preferably with the addition of .5% to 2% of copper or 130

upward to 5% of cobalt. For cyanide pots and salt baths the nickel should be increased advantageously to from 30 to 35 per cent as the highest resistivity to the effect of alkali

5 is obtained in an alloy having such proportions of the elements mentioned.

From the foregoing it will be observed that the proportion of nickel but not of chromium may be varied within a relatively wide range

10 so as to obtain the most desired properties of the alloy in each particular case. My invention resides, therefore, in the discovery of the peculiar characteristics of alloys of iron, nickel and chromium within the specified range of proportions and includes such alloys with an addition of elements which

15 modify the properties of the alloys without destroying the quality of endurance to deteriorating conditions at high temperatures.

20 Thus, while the maximum endurance is obtained with an alloy containing approximately 35 per cent of nickel, the greatest mechanical strength with a fair degree of endurance is obtained with an alloy containing approximately

25 20 per cent of nickel. Also while these alloys are not suitable for operations requiring malleability, a certain degree of toughness can be acquired by the addition of cobalt or copper or both without losing the advantages of the harder alloys with respect

30 to deterioration.

I have mentioned a few of the possible uses of the alloy and the particular compositions which are best adapted for employment in connection therewith. The effect of the several constituents has been described in more or less detail in order that the possibility of varying the properties of the alloy by increasing or diminishing the proportions

35 40 of the added constituents may be clear. Various changes may be made, therefore, in the details of the invention, particularly with

respect to the proportions of added constituents, without departing from the invention or sacrificing any of the advantages thereof. 45

I claim:

1. An alloy containing approximately 30% of chromium and 35% of nickel, the balance consisting principally of iron, said alloy being heat resistant in the presence of alkali 50 salts at high temperature.

2. A heat resisting structure adapted to withstand the action of alkali compounds at high temperatures, such structure being made of an alloy containing approximately 55 28 to 40% of chromium and 18 to 40% of nickel, the balance consisting principally of iron.

3. A heat resisting structure adapted to withstand the action of alkali compounds at 60 high temperatures, such structure being made of an alloy containing approximately 28 to 32% of chromium, about 18 to 40% of nickel, and the balance principally of iron.

4. A heat resisting structure adapted to 65 withstand the action of alkali compounds at high temperatures, such structure being made of an alloy containing approximately 28 to 40% of chromium and 18 to 40% of nickel, 70 the balance consisting principally of iron, said structure having a tough adherent oxidized coating.

5. A heat resisting structure adapted to withstand the action of alkali compounds at 75 high temperature, said structure being made of an alloy consisting mainly of chromium and iron, with a chromium content of from 28 to 40% sufficient to give heat resistance at or about 2000° F. and said alloy containing from 18 to 40% of nickel and being thereby 80 made heat resistant in the presence of alkali compounds.

In testimony whereof I affix my signature.

NOAK VICTOR HYBINETTE.